

Sept. 2, 1941.

C. KREUTZER

2,254,429

METHOD OF PRODUCING SELENIUM COATED ELECTRODES

Filed Dec. 16, 1938

*Fig. 1.*



*Fig. 2.*



*Inventor,*  
Conradin Kreutzer

*Glascock Downing & Sebold*  
By: Attorneys.

## UNITED STATES PATENT OFFICE

2,254,429

METHOD OF PRODUCING SELENIUM  
COATED ELECTRODES

Conradin Kreutzer, Nuremberg, Germany

Application December 16, 1938, Serial No. 246,237  
In Germany December 17, 1937

6 Claims. (Cl. 175—366)

This invention relates to a method of producing selenium rectifiers and selenium photo-cells.

In the production of selenium rectifiers and selenium photo-cells, in which selenium acts as a semi-conductor, considerable difficulties are encountered in obtaining the selenium in metallic modification from the metalloid in such a way as to produce a smooth surface or a surface of the desired form. If precautionary measures are not adopted during the process of conversion, the selenium tends to warp, and a rough honeycombed surface is produced, which is unsuitable for rectifiers or photo-cells. Investigations have shown that the reason for this condition resides in irregularity of the crystallisation process, the crystallisation centres being distributed irregularly over the surface.

It is an object of the invention to overcome this drawback, and this is accomplished by maintaining the selenium, during the conversion into the crystalline modification, in surface contact with a material, the only condition as regards the chemical nature of which is that the material does not enter into a chemical compound with the selenium and does not dissolve the selenium. The contact should be as complete as possible, and in particular the imprisonment of air should be avoided. Owing to the surface contact a large number of crystallisation centres are produced, which are distributed evenly over the layer of selenium, and from which the crystals develop in correspondingly even distribution towards the interior of the layer.

In this way there is obtained an evenly metallically crystallized selenium layer having a smooth surface, the form of which depends on the form of the base plate and on the form of the contacting surface.

In carrying out the invention the selenium is not fused onto the supporting electrode, but onto a material, such as aluminum, which does not enter into connection, or into conductive connection, with the selenium. The selenium can be applied to the material, which is preferably in the form of a foil, by a spraying operation, or it can be deposited thereon according to any of the conventional processes. A particularly convenient method has been found to consist in applying the amorphous selenium to the foil at a temperature which is below the fusing point of the crystalline selenium. The foil is then applied to the supporting electrode with the selenium downwards, preferably under a slight pressure to expel any air. The supporting elec-

trode merely requires to have a temperature below the fusing point of the crystalline selenium, or below 220° C. The foil, the amorphous selenium and the supporting plate are now connected together. The foil can be readily stripped off. This can be performed either after the forming or after the selenium has been allowed to cool.

The invention is illustrated by way of example in the accompanying drawing, in which

Fig. 1 is a sectional view of a metal foil showing the selenium applied thereto.

Fig. 2 is a sectional view illustrating the method of applying the selenium to an electrode.

In Figs. 1 and 2 there are shown the metal electrode 1a, the selenium 2a, and the contacting surface 3a, which in this case consists, for example, of a thin foil of aluminum. The selenium 2a is applied to the foil 3a, for example in a spraying operation, whereupon the foil with the layer 2a directed downwards is applied to the electrode 1a, which has either been heated or is then heated in the manner referred to. After the application the foil 3a is caused to bear intimately against the plate 1a, for example by passing a roller 4 over the same. After the cooling the foil 3a can be readily stripped off.

The method described offers considerable advantages as compared with known processes in which the selenium is fused onto the supporting electrode and in which it is necessary to raise the electrode to a temperature which is at least a few degrees above the fusing point of the selenium. In the latter case the selenium combines with the electrode to form selenide and the properties of the rectifier or the photo-cell are thus impaired.

What I claim as new and desire to secure by Letters Patent is:

1. The method of producing selenium coated electrodes which consists in applying a layer of amorphous selenium to a metal foil, arranging the layer of selenium carried by the foil in intimate contact with an electrode, subjecting the electrode and the foil to pressure to expel air from the selenium, maintaining the electrode and the foil at a temperature for converting the selenium into a crystalline state, cooling the selenium, and removing the foil.

2. The method of producing selenium coated electrodes which consists in spraying selenium onto an aluminum foil to provide a relatively thin layer of selenium thereon, arranging the layer of selenium carried by the foil over an electrode, rolling the foil to press the selenium into intimate contact with the electrode, heating

the selenium to convert the same into a crystalline state, cooling the selenium, and removing the foil.

3. The method of producing selenium coated electrodes which consists in, coating a metal foil with selenium to provide a layer thereon, arranging the selenium carried by the foil over an electrode, rolling the foil to provide intimate contact of the selenium with the electrode, and removing the foil.

4. The method of producing selenium coated metallic electrodes which consists in, applying a relatively thin layer of amorphous selenium to a metal foil, applying the selenium layer to a metallic electrode, heating the electrode to convert the selenium into a crystalline state, cooling the selenium, and removing the foil.

5. The method of producing selenium coated electrodes which consists in, applying selenium in an amorphous condition to a foil, arranging the selenium carried by the foil in contact with an electrode, heating the selenium to a temperature not exceeding 220° C., cooling the selenium, and removing the foil.

6. The method of producing selenium coated electrodes which consists in, spraying selenium in a finely divided condition onto a foil, heating an electrode to a temperature sufficient for rendering the selenium crystalline, applying the selenium carried by the foil onto the heated electrode, cooling the electrode, and removing the foil.

10  
15 CONRADIN KREUTZER.